

## UNITED STATES PATENT OFFICE

1,990,405

## METHOD OF MAKING BRIQUETTES

William L. Hoernle, Trenton, N. J.

No Drawing. Application August 22, 1930, Serial  
No. 477,193. Renewed July 10, 1934

6 Claims. (Cl. 44—23)

My invention relates to a novel and improved briquette and to the method of manufacturing it, and more particularly it relates to a briquette in which a novel type of binder is employed.

5 One object of my invention is to provide a water-resistant, odorless, and commercially smokeless briquette which is strong, hard and resistant to abrasion, and which can be manufactured at a relatively low cost.

10 Another object of my invention is to provide a coherent mass, or briquette, compounded of finely divided pulverulent materials and a binder whose melting point at the time that it is mixed with the finely divided materials is relatively low, but which during the process is converted into a non-coked binder of relatively high melting point.

15 Still another object is to provide a method of making briquettes in which it is possible to utilize the low melting tars and pitches which have not heretofore been considered applicable for use 20 as the main binding material.

Other objects will be apparent from a consideration of the specification and claims.

25 Briquettes have heretofore been manufactured by the use of pitches and tars of relatively high melting point, the use of which has required a considerable amount of heat to render them fluid and to keep them in this condition during the mixing preparatory to the pressing operations.

30 Difficulties are encountered for this reason, since the binder tends to set or solidify before a thorough mixing is obtained and before the briquettes are molded to the desired form. The low melting tars and pitches have not been used 35 as the main binding material, since they have been considered too soft and fluid for the purpose, due to the difficulty of handling the pressed briquette, their susceptibility to temperature changes near the melting point, and their tendency to disintegrate under firing conditions.

40 My invention is characterized by a new and improved method of adapting low melting tars and pitches for use in the manufacture of coherent masses, or briquettes. My invention contemplates the utilization as binders in briquette making of low melting tars and pitches, such for example, as those that melt below 125 degrees F., but which materials are capable of change under the influence of heat and oxygen to a non-coked 45 binder of relatively high melting point with the smoke-producing constituents removed. The change from the low melting tar to the high melting tar under the influence of heat and oxygen is termed herein "polymerization." The 50 term, however, is not necessarily used in its strict

sense, since it includes the change from a low melting tar to a high melting tar regardless of the phenomena involved, which may include an oxidation reaction as well as possibly one of reduction. The tar and pitches applicable for use according to the present invention may be designated as "low melting tars capable of polymerizing under heat and oxygen to form relatively high melting tars."

5 As examples of tars which may be used, "steam refined asphalt" and "water-gas tar" are mentioned. The former has a melting point (ball and ring) of 120-125 degrees F. and a penetration of 85-100 at 77° F. (100 grams, 5 seconds). It is usually obtained as a product or by-product of the distillation of asphaltic base crude oil. The "water-gas tar" has a melting point of 100 to 110 degrees F. and a specific gravity of 1.15-120. It is a product or by-product of the manufacture of carbureted water gas in a carbureted water-gas plant, and is usually extracted from the water-gas operation when a heavy oil commonly called "bunker C oil" is used in carburetion. It is applicable for use without further distillation or treatment. In addition to these two tars mentioned, various lignite, shale and coal tars are 20 applicable.

25 A wide variety of materials may be formed into briquettes by means of the tars herein contemplated. For example, the resulting coherent mass may be briquettes of ore, flue dust or concentrates; bricks or cores of sand or gravel or other finely divided pulverulent materials; or fuel briquettes of coal dust or coal fines. The term "finely divided particles" used throughout 30 the specification and claims includes granular, powdered, pulverized and other finely divided material.

35 In carrying out my invention, a briquette is molded to the desired size and shape, using as 40 the binding material a low melting tar of the characteristics previously described. The mass is then subjected to heat and oxygen which may be supplied by the air passing through the heat zone, or from any other source, for a sufficient 45 time to polymerize the low melting tar and to remove the smoke-producing constituents. In the heat and oxygen treatment, there is an exothermic reaction involved which automatically raises the temperature in the heat zone. The 50 binder throughout the briquette due to its gas-pervious nature is converted to one of high melting point and no appreciable amount of coking takes place. The cohesive qualities of the binder are, therefore, not destroyed. It is possible by 55

this treatment to raise the melting point of the tar in a marked manner. For example, it is possible to raise the melting point of "steam refined asphalt" from approximately 120-125 degrees F. to 250 degrees F., or even higher, depending somewhat on the time interval. The resulting briquette is hard, strong and resistant to abrasion. It is also water-resistant, odorless and commercially smokeless. The process allows 10 the use of the relatively cheap low melting tar in the manufacture of briquettes

In most cases a temperature of from 450 to 550 degrees F. and a time interval of from 30 to 90 minutes is sufficient to cause the desired polymerization if the air admitted and passed through the mass of briquettes is adequate to produce an oxidizing atmosphere in the heat zone. The size, weight and shape determine to some extent the time necessary to cause the polymerization. A pressure slightly above that of the atmosphere is preferably maintained and the use of preheated air is found to be advantageous. The percentage of tar relative to the finely divided material varies widely, depending upon the nature of the materials. In most instances the percentage of tar is between 3% and 15% by weight of the pulverulent material.

In a typical case the use of anthracite coal in finely divided form and "steam refined asphalt" of a melting point of 120-125 degrees F. and a penetration of 85 to 100 at 77° F. (100 grams, 5 seconds) will be described. The tar is employed in a percentage from 5% to 7% by weight of the coal particles. The two ingredients are thoroughly mixed either hot or cold as best suits conditions. In most instances it will be found desirable to raise the temperature of the coal and tar to a point where full advantage of the capillary attraction and affinity of the materials toward 30 each other is obtained, thus assuring a thorough and uniform mixture and the covering of each particle with a thin film of the tar. The briquettes are then formed under pressure by placing the mass in molds of the desired shape and size. The formed masses are placed on a perforated conveyor or wire screen to allow free passage of air and heat through the mass of briquettes. Preferably a conveyor is employed which travels in a horizontal plane or in an inclined plane of such inclination that the position of the soft briquettes is not changed until they are strong and hard, due to the polymerization. The briquettes are passed through a heat zone maintained at a temperature in the neighborhood 40 of 500 degrees F. for a period of 75 minutes, during which time a volume of preheated air is admitted in suitable quantities and passed through the heating zone to produce an oxidizing atmosphere of slightly greater pressure than that of the atmosphere of the surroundings. The briquettes are allowed to cool, and they will be found to have the qualities hereinbefore described.

Considerable modification is possible in the type of low melting tar used, in the ratio of tar to pulverulent material, and in the temperature, time and oxidizing conditions employed, since these factors depend to a large extent on the type of tar utilized, as well as on the size, weight and shape of the briquette, without departing 50 from the essential features of my invention.

I claim:

1. The process of making briquettes, which comprises covering finely divided particles to be agglomerated with a thin film of a tar whose melting point is below approximately 125 degrees

5 F. and which is capable of polymerization under simultaneously applied heat and oxygen to form a relatively high melting point tar with the smoke-producing constituents removed, forming the particles into gas-pervious masses of desired shape and size, and thereafter subjecting the formed masses at a temperature of at least 450° F. to intimate and direct contact with oxygen by passing a current of an oxygen-bearing gas through and around the masses during the heating, the heat and oxygen treatment being sufficient to cause polymerization to convert the low melting point tar into a tar of relatively high melting point with the smoke-producing constituents removed said treatment being insufficient to destroy the binding properties of the tar and to bring about coking thereof.

2. The process of making briquettes, which comprises covering finely divided particles to be agglomerated with a thin film of steam-refined asphalt whose melting point is below approximately 125 degrees F. and which is capable of polymerization under simultaneously applied heat and oxygen to form a relatively high melting point product with the smoke-producing constituents removed, forming the particles into gas-pervious masses of desired shape and size, and thereafter subjecting the formed masses at a temperature of at least 450° F. to intimate and direct contact with oxygen by passing a current of an oxygen-bearing gas through and around the masses during the heating, the heat and oxygen treatment being sufficient to cause polymerization to convert the steam-refined asphalt into a product of relatively high melting point with the smoke-producing constituents removed, said treatment being insufficient to destroy the binding properties of the asphalt and to bring about coking thereof.

3. The process of making briquettes, which comprises covering finely divided particles to be agglomerated with a thin film of a water-gas tar whose melting point is below approximately 125 degrees F. and which is capable of polymerization under simultaneously applied heat and oxygen to form a relatively high melting point tar with the smoke-producing constituents removed, forming the particles into gas-pervious masses of desired shape and size, and thereafter subjecting the formed masses at a temperature of at least 450° F. to intimate and direct contact with oxygen by passing a current of an oxygen-bearing gas through and around the masses during the heating, the heat and oxygen treatment being sufficient to cause polymerization to convert the water-gas tar into a tar of relatively high melting point with the smoke-producing constituents removed, said treatment being insufficient to destroy the binding properties of the tar and to bring about coking thereof.

4. The process of making briquettes, which comprises covering finely divided particles to be agglomerated with a thin film of a tar whose melting point is below approximately 125 degrees F. and which is capable of polymerization under simultaneously applied heat and oxygen to form a relatively high melting point tar with the smoke-producing constituents removed, forming the particles into gas-pervious masses of desired shape and size, and thereafter subjecting the formed masses to a temperature between 450 degrees F. and 550 degrees F. in the presence of an oxygen-bearing gas passed through and around the masses for a period of time between thirty and ninety minutes to cause polymerization to con-

vert the low melting point tar into a tar of relatively high melting point with the smoke-producing constituents removed, said heat and oxygen treatment being insufficient to destroy the binding properties of the tar and to bring about coking thereof.

5. The process of making briquettes, which comprises covering finely divided particles to be agglomerated with a thin film of steam-refined 10 asphalt whose melting point is below approximately 125 degrees F. and which is capable of polymerization under simultaneously applied heat and oxygen to form a relatively high melting point tar with the smoke-producing constituents 15 removed, forming the particles into gas-pervious masses of desired shape and size, and thereafter subjecting the formed masses to a temperature of approximately 500 degrees F. in the presence of an oxygen-bearing gas passed through and around the masses for a period of time of approximately 20 seventy-five minutes to cause polymerization to convert the steam-refined asphalt into a product of relatively high melting point with the smoke-producing constituents removed, said heat

and oxygen treatment being insufficient to destroy the binding properties of the tar and to bring about coking thereof.

6. The process of making briquettes, which comprises covering finely divided particles to be agglomerated with a thin film of water-gas tar whose melting point is below approximately 125 degrees F. and which is capable of polymerization under simultaneously applied heat and oxygen to form a relatively high melting point tar with the 10 smoke-producing constituents removed, forming the particles into gas-pervious masses of desired shape and size, and thereafter subjecting the formed masses to a temperature of approximately 500 degrees F. in the presence of an oxygen-bearing 15 gas passed through and around the masses for a period of time of approximately seventy-five minutes to cause polymerization to convert the low melting point tar into a tar of relatively high melting point with the smoke-producing constituents removed, said heat and oxygen treatment being insufficient to destroy the binding properties of the tar and to bring about coking thereof.

WILLIAM L. HOERNLE.